# EUROPEAN PATENT SPECIFICATION

(11) **EP 0 688 879 B1**
(45) Date of publication and mention of the grant of the patent: **04.02.1998**
(21) Application number: 95107446.7
(22) Date of filing: 17.05.1995
(51) Int. Cl.: C22C 9/00

(54) **High vacuum apparatus member and vacuum apparatus**
Hochvakuumanlage
Appareil à vide élevée

(30) Priority: 20.06.1994 JP 160596/94
(43) Date of publication of application: 27.12.1995
(73) Proprietor: Mitsubishi Materials Corporation, Chiyoda-ku, Tokyo (JP)
(72) Inventor: Ishida, Norikazu, c/o Chuo-kenkyusho, Omiya-shi, Saitama-ken (JP); Mae, Yoshiharu, c/o Chuo-kenkyusho, Omiya-shi, Saitama-ken (JP); Yajima, Kenji, c/o Chuo-kenkyusho, Omiya-shi, Saitama-ken (JP); Iwamura, Takuro, Chiyoda-ku, Tokyo (JP)
(74) Representative: Türk, Gille, Hrabal, Leifert

(56) References cited:
- EP-A- 0 296 596
- US-A- 4 717 436
- US-A- 5 077 005
- PATENT ABSTRACTS OF JAPAN vol. 13 no. 156 (C-585) ,14 April 1989 & JP-A-63 312934 (HITACHI CABLE LTD) 21 December 1988,
- PATENT ABSTRACTS OF JAPAN vol. 12 no. 122 (C-488) ,15 April 1988 & JP-A-62 243727 (HITACHI CABLE LTD) 24 October 1987,
- JOURNAL OF METALS, vol. 45, no. 3, March 1993 pages 68-70, RAJAINMAKI,H., KOLEHMAINEN,M.,HELENIUS,A. 'The Production and Application of Oxygen-Free Copper'
- METALL, vol. 44, no. 11, November 1990 pages 1067-1070, HELENIUS,A.,KOLEHMAINEN,M., RAJAINMAKI,H. 'Current and Future Uses of Oxygen-Free Copper'
- PATENT ABSTRACTS OF JAPAN vol. 12 no. 70 (C-479) ,4 March 1988 & JP-A-62 207834 (NIPPON MINING CO. LTD.) 12 September 1987,

## Description

The invention relates to the use of a material for the manufacture of high-vacuum appartuses such as power transmitter tubes, external anodes which also serve as vacuum containers for microwave tubes, vacuum deposition and sputtering apparatuses, klystrons, waveguides, acceleration cavity containers for accelerators, etc., from which hydrogen is easily removed by baking.

Conventionally, materials or members for the manufacture of high-vacuum apparatuses have generally been made of high-purity oxygen-free copper which satisfies required excellent electrical conductivity and thermal conductivity and includes low residual gas for preventing reduction in the degree of vacuum in a vacuum apparatus due to residual gas in the material from which the apparatus is made. Such low-residual-gas including high-purity oxygen-free copper is manufactured by degassing normal oxygen-free copper in a reducing or vacuum atmosphere, or by addition of phophorus for deoxygenation. High-purity oxygen-free copper produced in this manner contains 3 ppm or less of oxygen and 0.2 to 0.5 ppm of hydrogen, and vacuum apparatuses made of such high-purity oxygen-fee copper are subjected to dehydrogenation by vacuum annealing, called "baking", before use to guard against reduction in the degree of vacuum in a vacuum apparatus due to an out-gas from the material of the apparatus in a high vacuum.

Rajainmaki et al., 'The Production and application of oxygen free copper', JOM, (March 1993), 45, (3), pages 68-70 and Helenius, A. et al;, 'Current and Future uses of oxygen free copper', Metall, (Nov. 1990), 44, (11), pages 1067-1070, both describe the use of oxygen free copper in high vacuum apparatus.

However, even with dehydrogenation by baking prior to use of vacuum apparatuses manufactured using the aforementioned high-purity oxygen-free copper, certain problems result, since hydrogen contained in the high-purity oxygen-free copper is trapped by residual oxygen because of its strong affinity thereto, thus rendering the dehydrogenation more difficult. Consequently, when vacuum apparatuses manufactured using high-purity oxygen-free copper containing such oxygen-trapped hydrogen are used in a high vacuum, the residual hydrogen is gradually released and causes a reduction in the degree of vacuum.

The object of the present invention is the use of high-purity copper alloy material as high vacuum apparatuses which have, after baking, a reduced residual hydrogen content.

This object is solved in accordance with the present invention by the use of a high-purity copper material having the features of claim 1. Preferred applications of such material are subject matter of claims 2-3.

The inventors have conducted research aimed at producing a material suitable as vacuum apparatus member made of a copper alloy from which hydrogen is easily removed by baking, conventionally high-purity oxygen-free copper, which does not lead to a reduced degree of vacuum due to out-gassing hydrogen when used in a high vacuum, as well as a vacuum apparatus comprising such a vacuum apparatus member, and have found that a copper alloy prepared by adding 1 to 15 ppm of zirconium (Zr) to normal high-purity oxygen-free copper allows easy removal of hydrogen by baking and has a very low level of out-gassing of residual hydrogen from the material in a high vacuum, thus preventing reduction in the degree of vacuum.

The present invention has been accomplished on the basis of this finding, and is based upon the use of a material having a composition of high-purity oxygen-free copper with a purity of 99.99 wt% or greater, which contains 1 to 15 ppm of Zr and 3 ppm or less of oxygen as high vacuum apparatuses.

The material of the present invention allows easy removal of hydrogen by baking when it contains 1 to 15 ppm of Zr because, since Zr is an element with a very strong affinity for oxygen, residual trace oxygen in the copper alloy combines preferentially with Zr and is not dissociated therefrom even by heating during baking. Therefore, the residual trace oxygen in the high-purity copper alloy does not trap hydrogen, and thus the hydrogen is easily removed during baking.

However, a Zr content of less than 1 ppm is not preferred since this is insufficient for combining with the residual oxygen in the copper alloy, and conversely a Zr content of more than 15 ppm is not preferred since this reduces the hydrogen-removing effect during baking. The range of the Zr content is therefore established to be 1 to 15 ppm. A more preferred range of the Zr content is 3 to 10 ppm.

Since up to 3 ppm of oxygen in the copper alloy may combine with Zr in the above-mentioned range of 1 to 15 ppm, the oxygen content of the vacuum apparatus member of the present invention is preferably up to 3 ppm.

To manufacture vacuum apparatus members containing 1 to 15 ppm of Zr and 3 ppm or less of oxygen according to the present invention, first, electrolytic copper with a purity of 99.99 wt% or greater is melted in a melting furnace under constant protection with CO + N₂ gas, and the resulting molten metal is poured into a ladle while Zr is added to the flow of the molten metal for adjustement of the components to a prescribed composition.

The vacuum apparatus material and a method of producing it will now be explained in further detail by way of the following example and the attached drawings which is a schematic view of an apparatus for producing the vacuum apparatus material.

The apparatus shown in the drawings comprises a melting furnace 1, a spout 2, a tundish 3, an addition apparatus 4, a nozzle 5, a mold 6, a covering 7 of graphite particles and a sealing gas source 8 in order to produce an ingot 9.

First, electrolytic copper with a purity of 99.99 wt% or greater was prepared and melted in the melting furnace 1 in a CO + N₂ atmosphere. The resulting molten metal was passed through the spout 2 sealed with CO + N₂ gas and transported to the tundish 3, and Zr was added from the addition apparatus 4 to the flowing molten metal before it reached the tundish 3. The surface of the molten metal in the tundish 3 was covered with a layer of graphite particles 7 to prevent its oxidation. The molten metal was then fed from the tundish 3 via the nozzle 5 to the mold 6 which was also sealed with CO + N₂ gas, and an ingot 9 was obtained.

Table 1 below shows the composition of the ingot obtained in this manner as determined by measurement of the Zr and oxygen contents. Specimens of 25 mm length, 25 mm width and 8 mm thickness were cut out from the ingot, and further lathed to prepare vacuum apparatus members of the present invention (1 to 10 of Table 1), vacuum apparatus members for comparison (1 to 3 of Table 1) and vacuum apparatus members of the conventional art (1 to 3 of Table 1), each having a diameter of 20 mm and a thickness of 4 mm.

The vacuum apparatus material or members used in the present invention 1 to 10, vacuum apparatus members for comparison 1 to 3 and vacuum apparatus members of the conventional art 1 to 3 were subjected to baking for one hour at a temperature of 500 °C in a vacuum atmosphere of 266 x 10⁻⁵ Pa (2 x 10⁻⁵ Torr) and these baked vacuum apparatus members of the present invention, vacuum apparatus members for comparison and vacuum apparatus members of the conventional art were further charged into an out-gas measuring apparatus to measure the out-gassing rate of hydrogen gas in a high-vacuum atmosphere of 133 x 10⁻¹⁰ Pa (1 x 10⁻¹⁰ Torr) while at a temperature of 500 °C. The results are given in Table 1.

**TABLE 1**

| Vacuum apparatus member | | Composition | | | | Out-gassing rate (Torr·1/sec.·cm²) |
|---|---|---|---|---|---|---|
| | | Electrolytic copper purity (%) | Zr (ppm) | Oxygen (ppm) | P (ppm) | |
| Present invention | 1 | 99.998 | 3 | 1.8 | - | 1.33 x 10⁻¹¹ |
| | 2 | 99.998 | 4 | 2.0 | - | 2.17 x 10⁻¹¹ |
| | 3 | 99.998 | 3 | 1.7 | - | 2.34 x 10⁻¹¹ |
| | 4 | 99.998 | 1 | 0.7 | - | 6.75 x 10⁻¹² |
| | 5 | 99.998 | 7 | 1.8 | - | 8.98 x 10⁻¹² |
| | 6 | 99.998 | 12 | 2.0 | - | 1.10 x 10⁻¹¹ |
| | 7 | 99.998 | 14 | 2.7 | - | 2.14 x 10⁻¹¹ |
| | 8 | 99.998 | 6 | 1.2 | - | 9.77 x 10⁻¹² |
| | 9 | 99.998 | 11 | 1.5 | - | 7.29 x 10⁻¹² |
| | 10 | 99.998 | 10 | 2.0 | - | 1.01 x 10⁻¹¹ |
| Comparison | 1 | 99.998 | 7 | 5.0 * | - | 6.21 x 10⁻¹⁰ |
| | 2 | 99.998 | 0.6 * | 1.8 | - | 2.70 x 10⁻¹⁰ |
| | 3 | 99.998 | 18 * | 1.2 | - | 8.29 x 10⁻¹¹ |
| Conventional Art | 1 | 99.998 | - | 2.0 | 3.1 | 1.26 x 10⁻¹⁰ |
| | 2 | 99.998 | - | 1.5 | 2.8 | 8.92 x 10⁻¹¹ |
| | 3 | 99.998 | - | 2.5 | - | 1.94 x 10⁻¹⁰ |
| (Values marked with * are outside the range of the invention) | | | | | | |

The results shown in Table 1 demonstrate that the vacuum apparatus members of the present invention which contained 1 to 15 ppm of Zr and 3 ppm or less of oxygen all had lower values for the out-gassing rate of hydrogen gas in comparison with the vacuum apparatus members of the conventional art which did not contain Zr, and hence the hydrogen gas was more easily removed during the baking. In contrast, it was shown that the removal of hydrogen gas during baking was somewhat difficult in the case of the vacuum apparatus members for comparison 1-2 which were outside the ranges of 1 to 15 ppm of Zr and 3 ppm or less of oxygen. Also, as observed in the case of the vacuum apparatus member for comparison 3, a Zr content exceeding 15 ppm is not preferred as this causes more difficult removal of hydrogen gas during baking.

As explained above, use of a material as high vacuum apparatus members according to the present invention offers easier removal of hydrogen during baking than vacuum apparatus members of the ceonventional art, and therefore it produces the excellent industrial effect with superior performance.

## Claims

1. Use of high-purity copper material containing, prior to annealing (baking), hydrogen, 3 ppm or less of oxygen and 1 to 15 ppm of Zr and having a purity of 99,99 weight % or higher as a material for the manufacture of high-vacuum apparatuses.

2. The use of the material according to claim 1 containing 3 to 10 ppm of Zr for the same purpose as in claim 1.

3. The use of the material according to any of claims 1 or 2 for constructing power transmitter tubes, external anodes which also serve as vacuum containers for microwave tubes, vacuum deposition and sputtering apparatuses and acceleration cavity containers for accelerators.

## Patentansprüche

1. Verwendung eines hochreinen Kupfermaterials, das vor dem Glühen (Wärmebehandlung) Wasserstoff, 3 ppm oder weniger Sauerstoff und 1 bis 15 ppm Zr enthält und eine Reinheit von 99,99 Gew.-% oder höher besitzt, als Material für die Herstellung von Hochvakuumapparaturen.

2. Verwendung des Materials nach Anspruch 1, das 3 bis 10 ppm Zr enthält, für den gleichen Zweck wie in Anspruch 1.

3. Verwendung des Materials nach Anspruch 1 oder 2 zur Herstellung von Energietransmitterröhren, Außenanoden, die auch als Vakuumbehälter für Mikrowellenröhren dienen, Vakuumbeschichtungsapparaturen, Kathodenzerstäubungsapparaturen und Beschleunigungshohlraumbehältern für Beschleuniger.

## Revendications

1. Utilisation d'un matériau de cuivre de grande pureté contenant, avant recuit (cuisson), de l'hydrogène, 3 ppm ou moins d'oxygène et 1 à 15 ppm de Zr et ayant une pureté de 99,99 % en poids, ou plus, en tant que matériau pour la fabrication d'appareils à vide poussé.

2. Utilisation du matériau selon la revendication 1 contenant de 3 à 10 ppm de Zr dans le même but que selon la revendication 1.

3. Utilisation du matériau selon l'une quelconque des revendications 1 ou 2 pour construire des tubes transmetteurs de puissance, des anodes externes qui servent également comme récipient à vide pour des tubes à micro-ondes, des appareils de dépôt sous vide et de pulvérisation cathodique et des récipients de cavité d'accélération pour accélérateurs.
